

## UNITED STATES PATENT OFFICE

2,431,191

COBALT RESINATE AND METHOD OF  
PRODUCING

Paul R. Mosher, Wilmington, Del., assignor to  
Hercules Powder Company, Wilmington, Del.,  
a corporation of Delaware

No Drawing. Application September 4, 1941,  
Serial No. 409,534

12 Claims. (Cl. 260—105)

1

This invention relates to the production of cobalt resinate and more particularly to fused cobalt resinate of improved characteristics and to the method of production thereof.

By reaction of wood or gum rosins with suitable cobalt compounds, cobalt resinate have been prepared containing an amount of cobalt in combined form up to the theoretical cobalt content of the neutral diresinate. Production of the cobalt resinate from such rosins has been carried out either by fusion of the rosins with suitable cobalt compounds or by a double decomposition procedure involving treatment of a water-soluble salt of the rosins with a soluble cobalt salt. By the precipitation method cobalt resinate containing up to the theoretical cobalt content for the neutral diresinate have been prepared. By the fusion method, on the other hand, it has been impossible to introduce more than a small amount of cobalt due to the fact that the fusion mixture sets to a solid mass or "blocks," and consequently only acid resinate of low cobalt content have been capable of production by the fusion method. The blocking phenomenon encountered is the result of a change of the fluid mix into a solid, non-homogeneous, partially crystallized, opaque and relatively insoluble mass.

It is an object of this invention to provide cobalt resinate of higher cobalt content than has heretofore been possible.

It is another object to provide fused cobalt resinate of high cobalt content which possess many improved characteristics.

It is a further object to provide a method of producing fused cobalt resinate of high metal content.

Other objects of the invention will appear hereinafter.

The above objects may be accomplished in accordance with this invention by fusing a cobalt compound capable of reaction with rosins, at a temperature in the range of about 200° C. to about 340° C. with a rosins which has been previously subjected to a heat treatment at a temperature in the range of about 250° C. to about 350° C. until the optical rotation of the rosins in the solid state has reached the range of about +20° to about +60° and preferably from about +30° to about +50°. It has been found in accordance with this invention that by first subjecting rosins to a heat treatment to increase its optical rotation to at least +20° and then fusing with a reactive cobalt compound at the above temperatures all blocking difficulties are avoided and resinate having a cobalt content above

2

the theoretical cobalt content of the cobalt diresinate are readily obtained. Thus, in accordance with this invention, cobalt resinate having a cobalt content greater than the equivalent combining proportion of the rosins based on its acidity and as high as 19% by weight are provided by fusing the heat-treated rosins with a sufficient amount of a reactive cobalt compound to give the required combining proportion of cobalt. The theoretical cobalt content of a diresinate prepared from a rosins of theoretical acid number is 8.93%. This amount of cobalt thus represents the maximum obtainable in a resinate by the precipitation method and far exceeds the amount capable of introduction by a fusion procedure.

In carrying out the process of the invention a heat-treated rosins having a specific optical rotation from about +20° to about +60° and preferably from about +30° to about +50° is reacted with a cobalt compound capable of reaction therewith to provide a salt. Such a compound may be a basic cobalt compound or it may be a cobalt salt of a volatile weak acid, or any other cobalt compound which under the fusion conditions liberates its cobalt. Suitable cobalt compounds are, for example, cobalt acetate, cobalt formate, cobalt lactate, cobalt butyrate, cobalt oxide, mixtures of cobalt oxide with a fatty acid cobalt salt as the acetate, mixtures of cobalt oxide with a fatty acid as acetic acid, etc. In using cobalt oxide it is usually desirable to employ it in admixture with a fatty acid salt or a fatty acid since the reactivity of the oxide alone in some cases is not sufficient to provide homogeneous resinate. If desired, a small amount of calcium acetate or other fatty acid salt of calcium or a fatty acid salt of zinc, lead, manganese, etc., may be employed with cobalt oxide to facilitate reaction of the latter. When such auxiliary agents are used, they combine partially with the heat-treated rosins also. The amount of such auxiliary agent necessary will only be a small amount, as for example from about 0.5% to about 2% by weight based on the rosins.

The fusion reaction of the invention is performed by heating the heat-treated rosins of the above characteristics to a temperature in the range of about 200° C. to about 340° C. and adding the cobalt compound either gradually or at one time, preferably while agitating the mixture. Foaming accompanies the reaction and agitation serves to hold the foaming to a minimum. The foaming is more severe at the lower temperatures and the reaction is also slower. At temperatures

above about 320° C. the reaction is vigorous but the yield becomes diminished due to volatilization of light ends from the heat-treated rosin. Preferable temperatures for the reaction therefore are from about 230° C. to about 320° C.

The time of reaction required to form the novel resinate is dependent on the temperature employed, the particular cobalt compound used, the degree of agitation and the amount of metal being introduced, as well as on other factors. Thus, the reaction time may be varied from about 10 minutes to several hours. Presence of an inert atmosphere, such as may be provided by carbon dioxide, nitrogen, etc., prevents oxidation of the heat-treated rosin and the resinate at the elevated temperatures employed and is therefore desirable, though not essential.

The heat-treated rosin which has been found to be useful in carrying out this invention may be obtained by methods well known in the art. It has been recognized that heating of a natural rosin, as wood or gum rosin, at temperatures of 250° C. to 350° C. brings about both chemical and physical transformations in the rosin. The heat treatment has been carried out both in the presence and absence of an inert atmosphere and the same fundamental changes appear to occur. The specific optical rotation increases in the positive direction as the heat treatment progresses. The crystallizing tendencies of the rosin also decrease and the rosin becomes bleached in color as the heat treatment is prolonged. It is not known which of these chemical and physical changes is responsible for the different behavior of the rosin in the production of cobalt resinate by the fusion method. It is probably a combination of each of the transformations which provides such a pronounced effect in resinate formation.

The most accurate means of defining the heat-treated rosins which possess the necessary characteristics for practice of this invention is by means of the specific optical rotation, as measured on the solid rosin. Thus, it has been found that when the optical rotation of the heat-treated rosin, as measured on the solid rosin, reaches +20° the characteristic of forming cobalt resinate of high cobalt content by a fusion process without blocking is first observed. This characteristic is most pronounced when the heat treatment has been sufficient to raise the optical rotation to +30°. When the optical rotation is above +30° the heat-treated rosin will be substantially non-crystalline and non-crystallizing. It will also be substantially lighter in color than the rosin from which it was produced, thereby providing an improvement in the color of the resinate. The heating time required to provide the desired changes in the rosin will vary with the particular temperature employed. It may be from about five minutes to as long as 8 hours.

The novel cobalt resinate described in accordance with this invention will be sharply differentiated from prior art cobalt resinate in their higher cobalt contents. They will thus be more desirable in the various uses of cobalt resinate, as in driers for paints and varnishes, in printing inks, etc. They will be clear, homogeneous and substantially neutral resins having a deep purple color.

The following specific examples illustrate the various embodiments of the invention:

#### Example I

A heat-treated wood rosin was prepared by subjecting N wood rosin to a temperature of 310

to 315° C. until its optical rotation reached +40°. The heat-treated rosin so obtained had an acid number of 133 and a melting point (drop) of 74° C. Sixty-nine parts by weight of the heat-treated rosin were melted and heated to a temperature of 220° C. Thirty-seven parts by weight of cobalt acetate were added to the molten rosin in small portions at a time with continuous agitation, allowing time between each addition for the reaction to become complete, as evidenced by the subsiding of foaming and evolution of acetic acid. The temperature was raised gradually during the addition to a maximum of 250° C. The total time of addition was 20 minutes, after which the resinate was cooled. The cooled cobalt resinate was a clear, homogeneous resin of purple color having a drop melting point of 137° C. and a cobalt content of 11%.

#### Example II

One hundred parts by weight of the heat-treated wood rosin used in Example I were melted and heated to a temperature of 270° C. One hundred parts by weight of cobalt acetate were then added in small portions at a time with agitation, allowing time for the reaction to become complete between each addition. The temperature was raised gradually to 305° C. during the addition, which required 50 minutes. The cooled cobalt resinate obtained was a clear, homogeneous, resinous solid of purple color having a cobalt content of 19% and a melting point (drop) of 175° C.

#### Example III

35 A heat-treated gum rosin was prepared by subjecting WW gum rosin to a heat treatment at a temperature of 310 to 315° C. until the optical rotation reached +41°. The heat-treated rosin so obtained had an acid number of 127 and a melting point (drop) of 82.5° C. One hundred parts by weight of the heat-treated gum rosin were melted and heated to a temperature of 240° C. Eighty-six parts by weight of cobalt acetate were then added in small portions at a time with agitation, allowing the reaction to become complete between each addition. The temperature was raised gradually during the addition to a maximum of 330° C. The total time of addition was 35 minutes. The cobalt resinate obtained after cooling was a clear homogeneous rosin-like product having a cobalt content of 17% and a melting point (drop) of 163° C.

55 Thus it will be apparent from the above description and illustrative examples that by means of this invention a process is provided for obtaining cobalt resinate of higher metal content than heretofore possible. The process itself provides an important advance in the art of preparation of cobalt resinate. By means of the improved process all blocking difficulties formerly encountered in preparation of cobalt resinate by a fusion process have been overcome, and fused cobalt resinate of greater utility due to their higher metal content are made available.

60 It will be understood that the details and examples hereinbefore set forth are illustrative only and that the invention as herein broadly described and claimed is in no way limited thereby.

65 What I claim and desire to protect by Letters Patent is:

1. A cobalt resinate of a heat-treated rosin, said resinate having a cobalt content greater than the equivalent combining proportion of the rosin based on its acidity but not in excess of about 19% by weight, said heat-treated rosin being the



has reached the range of about  $+20^{\circ}$  to about  $+60^{\circ}$ .

PAUL R. MOSHER.

REFERENCES CITED

The following references are of record in the file of this patent:

UNITED STATES PATENTS

| Number    | Name                  | Date          |
|-----------|-----------------------|---------------|
| 1,884,407 | Romaine               | Oct. 25, 1932 |
| 2,072,628 | Brennan et al.        | Mar. 2, 1937  |
| 2,138,183 | Littman               | Nov. 29, 1938 |
| 2,157,767 | Long                  | May 9, 1939   |
| 2,175,491 | Stresen-Reuter et al. | Oct. 10, 1939 |

| Number      | Name              | Date          |
|-------------|-------------------|---------------|
| 2,205,458   | Pragoff           | June 3, 1942  |
| 2,225,246   | Hasselstrom       | Dec. 17, 1940 |
| 2,241,341   | Ender             | May 6, 1941   |
| 5 2,247,399 | Palmer et al. (1) | July 1, 1941  |
| 2,346,993   | Palmer et al. (2) | Apr. 18, 1944 |
| 2,346,994   | Palmer et al. (3) | Apr. 18, 1944 |

OTHER REFERENCES

|    |                                                                                       |
|----|---------------------------------------------------------------------------------------|
| 10 | Ruzicka, Helvetica Chimica Acta, vol. 5, 1922, page 338.                              |
| 15 | Du Pont et al., Chimie et Industrie, Special Number, pages 552 to 554, vol. 19, 1929. |
|    | Fleck et al., Journ. Amer. Chem. Soc., vol. 61, No. 2, page 247.                      |